

## UNITED STATES PATENT OFFICE

2,656,316

## LUBRICATING OILS CONTAINING METAL SALTS OF A CONDENSATION PRODUCT OF A SUBSTITUTED PHENOL AND A VINYL COMPOUND

Loren L. Neff, Long Beach, Calif., assignor to Union Oil Company of California, Los Angeles, Calif., a corporation of California

No Drawing. Application July 17, 1950,  
Serial No. 174,367

15-Claims. (Cl. 252—33.4)

1

This invention relates to lubricating oil addition agents having exceptional anti-corrosion and detergent characteristics when added to mineral lubricating oil, and to lubricating oils containing such addition agents with and without supplemental detergents. More particularly, the invention relates to oil-soluble metal salts of the condensation products obtained by condensing hydrocarbon substituted phenols with vinyl compounds and to lubricating oils containing such metal salts.

The present trend in internal combustion engines, particularly of the diesel engine type, is in the direction of higher compression ratios, higher operating temperatures and thus higher horsepower output per unit weight of the engine. Moreover, it is the trend to operate engines of this type for longer periods without oil change so that oils which are satisfactory for use in the present-day high output diesel engines, for example, must have not only an initially high detergent and initially high anti-corrosion characteristics but these properties must be retained under severe conditions of use for relatively long periods of use in an engine. To further complicate the preparation of a satisfactory oil for the lubrication of such engines the fuels available often contain higher proportions of sulfur than those which have been used in the past and it is well recognized that high sulfur fuels tend to produce corrosive conditions in an engine which must be overcome by the lubricating oil employed, otherwise not only does corrosion take place in the engine but wear rates are sufficiently high that frequent overhaul and replacement of parts becomes necessary, thereby unduly increasing engine operation cost.

In order to prepare oils which may be used in engines of the character described it has been the practice to merely increase the percentage of additive materials which have been used in the past in ordinary diesel engines, automotive engines and the like, hoping to gain the extra protection necessary by the use of these larger proportions.

It is an object of this invention to prepare a lubricating oil which will operate satisfactorily in internal combustion engines and particularly in the high output diesel engines over relatively long periods of service. It is another object to prepare such lubricating oils which will protect engines of this type operating under severe conditions even while using a fuel containing as high as 1% or more of sulfur.

It is found that these and other objects can

be obtained by adding to mineral lubricating oil relatively small amounts of an oil-soluble metal salt of the condensation product of a hydrocarbon substituted phenol and a vinyl compound of the type described hereinbelow.

Thus the invention resides in lubricating oils containing between about 0.05% and about 10% or as high as about 20% by weight of an oil-soluble metal salt of the condensation product obtained by condensing a hydrocarbon substituted phenol wherein the hydrocarbon substituent or substituents contain between about 4 and about 30 carbon atoms with a vinyl compound of the class consisting of vinyl ethers and vinyl esters of hydrohalogen acids and fatty acids. These condensation products are acidic and capable of reacting with metal bases, as for example, metal oxides, hydroxides and carbonates, under appropriate conditions to form the corresponding metal salts. The term "hydrohalogen acids" is used herein in its usual sense and includes hydrogen chloride, hydrogen bromide, hydrogen fluoride and hydrogen iodide. These acids may also be termed hydrogen halides.

A typical oil-soluble metal salt is produced by reacting approximately one molecular proportion of octyl phenol with one molecular proportion of vinyl acetate. The phenol and acetate are dissolved in about 2 parts by volume of a petroleum naphtha and to the solution is added about 2 parts by volume of a condensation catalyst, e.g. sulfuric acid. The catalyst is added slowly and the temperature of the reaction mixture is maintained at a point such that the vinyl acetate is not vaporized excessively. Preferably, because of the low boiling point of vinyl acetate, the reaction is conducted under a reflux condenser. Under any circumstance, by maintaining a temperature in this instance between about 30° C. and about 40° C., the reaction proceeds rapidly and smoothly and is complete in approximately 1.5 to 2 hours. Since the reaction is exothermic, completion of the reaction can be determined by following the temperature of the reaction mixture. Thus, whereas during the early part of the reaction cooling is necessary in order to maintain the temperature within the range of 30° C. to 40° C., toward the end of the reaction heat may be necessary in order to maintain this temperature. Following the completion of the reaction the product is cooled and water washed until free of mineral acid. Upon evaporation of the solvent naphtha employed there remains a semi-solid resin having a brownish color. The resin

may be converted into its metal salt, as for ex-

ample the barium salt, by treatment of a solvent solution, as for example a naphtha, or a hydrocarbon lubricating oil solution of the resin with barium hydroxide octahydrate or with anhydrous barium hydroxide, in which latter case it is necessary to add small amounts of water during the neutralization. Where the metal salt is the desired product, the solvent solution of the condensation product is mixed with the desired metal base and, after neutralization and elimination of water, the solvent is evaporated leaving the metal salt of the condensation product. The barium salt of the above condensation product is a semi-solid to solid resin of brownish color. Where it is desirable to prepare a lubricating oil concentrate of the metal salt of the condensation product the neutralization is preferably effected in mineral oil solution. In this case the condensation product or the solvent solution of the condensation product is dissolved in about 1 to about 5 volumes of mineral oil and the desired metal base and water is added. The resulting product is agitated and heated sufficiently to effect complete neutralization and subsequently filtered to remove solid impurities. The resulting product will be referred to as an oil concentrate of an oil-soluble metal salt of the condensation product of a hydrocarbon substituted phenol and a vinyl compound of the class described.

Hydrocarbon substituted phenols which are useful in the preparation of the oil-soluble metal salts of this invention include the phenols having alkyl, cycloalkyl, aryl, aralkyl and alkaryl substituents. The substituents may be in the ortho-, meta- or para-positions. Preferably the compound will have either an ortho- and a para-position free of substituents, or if the para-position is substituted then preferably both ortho positions should be free of substituents. Alkyl substituents include the butyl, amyl, iso-amyl, hexyl, heptyl, octyl, lauryl, cetyl and like radicals. These radicals may be normal or branched chain groups and the phenol may contain one or more of these substituents. Moreover, the alkyl substituents include the so-called wax radicals, i. e. radicals derived from paraffin wax which may contain as high as 30 or more carbon atoms. Wax phenols are well known in the art and may be prepared by reacting phenol with chlorinated paraffin wax in the presence of a Friedel-Crafts catalyst. Cycloalkyl substituents include cyclohexyl, methylcyclohexyl, cyclopentyl, methyl, ethyl and propyl cyclopentyl radicals and the like. Aryl radicals include the phenyl radical, as for example phenyl phenol. Aralkyl radicals include the benzyl radical and thus benzyl phenol. Alkaryl radicals include the radicals such as methylphenyl, ethylphenyl and the like.

Vinyl compounds which are useful in preparing the condensation products are the lower molecular weight vinyl ethers, as for example divinyl ether, vinyl ethyl ether, vinyl propyl ether and the like and vinyl esters. The vinyl esters include the vinyl hydrohalogen acid esters, as for example vinyl chloride, vinyl bromide and vinyl iodide and the lower molecular weight carboxylic acid esters, as for example vinyl acetate, vinyl propionate, vinyl butyrate and the like. Generally the carboxylic acid radical present in the ester will contain 1 to 5 or 6 carbon atoms and preferably 2 to 4 carbon atoms.

The molar ratio of hydrocarbon substituted phenol to vinyl compound to be used in preparing desirable condensation products will be be-

tween about 0.5 and about 3 to 1. Preferably this molar ratio will fall between about 0.8 and about 2 to 1. Particularly satisfactory results have been obtained using approximately equal molecular proportions of hydroxy compound and vinyl compound.

Catalysts or condensation agents which may be employed and which serve to effect the desired condensation reaction include the acid catalysts, as for example sulfuric acid and phosphoric acid, as well as the Friedel-Crafts type catalysts including aluminum chloride, boron trifluoride, zinc chloride and the like. In the case of boron trifluoride, this compound is generally employed in the form of its complex with diethyl ether. The complex is known as boron trifluoride etherate and has a boiling point of about 125° C. The amount of catalyst to be employed will generally be between about 0.5% and 10% by weight of the total reactants. However, as much as 20% may be employed if desired, with satisfactory results.

Although the condensation reaction will take place in the absence of solvent or diluent, it is generally desirable to employ a solvent during the condensation reaction. Solvents which may be employed include those which do not react with phenols or with the vinyl compounds under the conditions of condensation. Such solvents include the hydrocarbon naphthas or thinners, aromatic solvents, as for example benzene, toluene, and xylene, and the like as well as chlorinated solvents such as chloroform, carbon tetrachloride and the like. Also, the condensation is satisfactorily effected using mineral oil as the solvent or diluent. Thus, the solvent can be the oil to be used in the preparation of the final lubricating oil composition. The amount of solvent or diluent to be employed may be widely varied, although generally between 0.5 and 5 volumes of solvent per volume of reactants is found to give satisfactory results.

The temperature of reaction will depend upon the reactants involved but will generally be between about -20° C. and about 150° C. and preferably between about 0° C. and about 100° C. The temperature employed will depend to some extent upon the volatility of the vinyl compound employed. With the more volatile compounds, as for example vinyl chloride, lower temperatures are generally preferred and in this case particularly pressures of 1 to 3 or 4 atmospheres may be employed in order to maintain the reactants in solution or in liquid condition.

The time of reaction is dependent upon the particular reactants and upon the temperature and catalyst employed, although generally it is found that between about 1 hour and 4 or 5 hours suffice to effect the desired extent of condensation. However, entirely satisfactory condensation products have been prepared when the reaction conditions were maintained for as long as 24 hours. Products so obtained are found to be oil-soluble and metal salts derived from the condensation products are also oil-soluble.

The metals to be employed in preparing metal salts are preferably the polyvalent metals, although the monovalent alkali metals are satisfactory in some instances. Thus the sodium, potassium and lithium salts are found to be oil-soluble and have the desired characteristics when added to mineral lubricating oils. Of the polyvalent metals, the alkaline earth metals calcium, magnesium, barium and strontium are particularly effective. However, the zinc, lead and

aluminum salts are suitable and in some cases chromium, iron, nickel, cobalt, mercury, tin and other polyvalent metal salts have utility and are to be considered part of this invention, although this latter group of polyvalent metal salts are not to be considered equivalent to the alkaline earth metals and zinc, lead and aluminum salts.

In preparing metal salts of the condensation products a solvent solution or a lubricating oil solution of the condensation product is heated with the desired metal base, i. e. oxide, hydroxide or carbonate, in the presence of a small amount of water or in the presence of a small amount of alcohol. The mixture is agitated and heated to eliminate water and effect neutralization. In the case of the more weakly basic metals the metal salt is preferably made by a method involving first preparing the alkali metal salt, as for example the sodium salt, and subsequently metathesizing the alkali metal salt with an inorganic salt of the desired metal. This metathesis is carried out in alcoholic solution in order to prevent hydrolysis which would occur in aqueous solution. Methods of metathesizing weak acid salts are well known in the art and therefore need no further description here. This same method of preparation may be employed in producing any of the polyvalent metal salts if so desired.

In preparing finished lubricating oils the oil-soluble metal salts or the oil concentrates thereof, produced as indicated above, are added to mineral lubricating oil in proportions such that the final oil will contain between about 0.05% and about 20% and preferably between about 0.5% and 10% by weight of the salt. Although no difficulty is encountered in preparing oil solutions because of the ready oil-solubility or oil-dispersibility of these compounds, the solutions are generally prepared by heating the oil containing the metal salt to a temperature of 100° C. to 150° C. and agitating the solution to effect rapid and complete solution and/or dispersion. Lubricating oils which may be employed include substantially all types of mineral lubricating oils. Thus the oil may be one having a viscosity index of 0 or even lower or it may be a paraffinic type oil having a viscosity index in the neighborhood of 100. Particularly satisfactory results have been obtained using a solvent treated Western paraffinic mineral lubricating oil having a viscosity index of between about 85 and 95.

Although lubricating oils containing the additive of this invention as the only additive material are particularly effective, it is often necessary, particularly where the oil is to be used under severe service conditions, to incorporate in the oil relatively small amounts of a supplemental detergent. It is found, for example, that oil-soluble metal sulfonates and particularly the oil-soluble metal salts of mahogany sulfonic acids obtained by treating lubricating oil fractions of petroleum with sulfuric acid,  $SO_3$  or chlorosulfonic acid, which methods of preparation are well known in the art, appear to cooperate with the additives of this invention to produce outstanding lubricating oils. Thus by adding between about 0.5 and 5% by weight of a metal petroleum sulfonate it is found that the detergency of the oil is improved without adversely affecting the anti-corrosion or anti-oxidation characteristics of the oil.

Another detergent which appears to cooperate with the additives of this invention is a modified sulfonate prepared by heating an oil-soluble

metal petroleum sulfonate with an inorganic base to solubilize the base in the sulfonate. Thus, mahogany sulfonic acids may be reacted with inorganic bases as, for example, with metal oxides, hydroxides, carbonates and bicarbonates, to produce oil-soluble complexes containing a ratio of equivalents of metal to sulfonic acids between 1.1 to 1 and 3 or more to 1 and these materials are found to impart exceptional detergency characteristics to lubricating oils containing the condensation product salts of this invention. Such oil-soluble complexes of sulfonic acids and metal hydroxides, oxides, carbonates and the like which may be employed together with the additive of this invention are those described by Mertes in U. S. Patents Nos. 2,501,731 and 2,501,732.

Three different engine tests have been employed in the evaluation of lubricating oils containing the oil-soluble metal salts of this invention. These tests have been carried out in Lauson single cylinder engines, standard 6-cylinder Chevrolet engines and a single cylinder Caterpillar diesel standard test engine. The tests are referred to as the Lauson engine test, the Chevrolet engine test and the Caterpillar test, respectively.

Tests in the Lauson single cylinder test engines are carried out in such a manner that the oil is subjected to severe service conditions. This test is employed to determine the corrosion tendencies of the oil and to determine the tendency for the oil to deposit resinous and lacquer-like materials in the engine. In carrying out the Lauson engine test the engine is operated for a total of 60 hours under a load of about 3.5 horsepower, with a coolant temperature of about 295° F. and an oil temperature of about 280° F. At the end of the test the cleanliness of the engine is observed and the oil is given a numerical detergency rating between 0% and 100%, where 100% indicates a perfectly clean engine. Thus, a detergency rating of 100% would indicate that during the test with a given oil there were substantially no lacquer or varnish-like deposits within the engine. The corrosivity of the oil is measured by determining the loss in weight of corrosion-sensitive copper-lead bearings during the period of test. Generally, the bearings are removed and weighed after 20, 40 and 60 hours of operation.

In those cases in which corrosion is extremely severe and there appears to be danger of engine failure due to excessive corrosion of the bearings as indicated by an examination made at the 40-hour period, the copper-lead bearings are replaced with Babbitt bearings in order to complete the 60-hour test. The results of such engine tests are shown in connection with some of the examples presented hereinbelow.

In the Chevrolet engine test the engine is operated under a load of about 30 horsepower with a coolant temperature of about 200° F. and an oil temperature of about 280° F. This test is used to evaluate corrosivity of the lubricant. The loss in weight of copper-lead bearings is determined after 36 or more hours of operation.

In the Caterpillar test which is employed to determine the detergency of an oil, i. e., the ability of the oil to prevent lacquering of the engine, the engine is operated for a period of 240 hours under a load of about 19.8 horsepower with a coolant temperature of about 175° F. and an oil temperature of about 145° F. The fuel employed is a diesel fuel containing 1% by weight of sulfur. After 120 hours and at the end of the test a nu-

merical "detergency rating" is assigned. The method of rating is similar to that employed in the Lauson engine test and 100% indicates a completely clean engine. Also the volume of carbon present in the top ring groove behind the ring is determined and this result is expressed as percent by volume of the space behind the top ring at the start of the test.

The following examples illustrate some modifications of the invention, however it is to be realized that various modifications of the described methods of preparation and the described condensation product salts come within the scope of the invention.

*Example I*

A 438 g. (2.12 mols) portion of octylphenol is dissolved in 710 ml. of a light paraffine naphtha and to this solution is added 182 g. (2.11 mols) of vinyl acetate. This mixture is placed in a flask equipped with a stirrer, thermometer and reflux condenser.

Sulfuric acid (98% concentration) is added drop-wise through the reflux condenser until a total of 23.3 ml. (approximately 0.42 mols) has been added. During the initial addition the temperature rises to a point of rapid reflux (about 68° C.), and the addition is continued at a rate such that refluxing continues. Following the addition of the sulfuric acid the mixture is heated at its reflux temperature for 2.5-3 hours and then cooled.

The product is washed with water until free of acid and then dissolved in 2500 g. of an SAE 30 solvent extracted Western mineral lubricating oil and the mixture heated to 140° C. to vaporize the paraffinic naphtha used as solvent in the initial reaction.

The product is converted into its barium salt by adding 187 g. of anhydrous barium hydroxide and 350 ml. of water. The water is added drop-wise at 140° C. The resulting mixture is heated to 175° C., diluted with an additional 1000 g. of the same lubricating oil and filtered while hot using a filter aid. This product is an oil concentrate containing approximately 15.4% by weight of the barium salt of the condensation product of octylphenol with vinyl acetate. This product without further dilution operates satisfactorily in a Lauson engine, giving a high detergency and very low bearing weight losses.

A lubricating oil is prepared by dissolving 21.8 parts by weight of the above oil concentrate and about 3.7 parts by weight of an oil concentrate of calcium petroleum sulfonate in 74.5 parts by weight of the same SAE 30 mineral lubricating oil described above. The resulting oil containing approximately 3.4% by weight of the barium salt and having a calcium sulfate ash due to calcium sulfonate of approximately 0.24% is tested in a Caterpillar engine as described above, using a fuel containing 1% of sulfur. This oil has a detergency rating at 120 hours of 96% and at 240 hours of 96%. The percent of carbon in the top ring groove is 13 at 120 hours and 11 at 240 hours.

In comparison, the base oil without additives cannot be tested in this engine using a 1% sulfur fuel for the reason that the deposits are so great as to cause piston and ring sticking at far less than 120 hours to such an extent that it is impossible to complete the test. The base oil, i. e. the oil without additives, run in the same engine using a low sulfur fuel has a detergency rating of approximately 55% at 120 hours.

Tests on the base oil, on the oil concentrate as produced above, and on the oil prepared for testing in the Caterpillar test engine are as follows:

| 5  | Base Oil                          | Concentrate (15.4% of Barium Salt) | Oil Tested in Caterpillar Engine |
|----|-----------------------------------|------------------------------------|----------------------------------|
| 10 | Viscosity, SSU at:<br>100° F..... | 509.6                              | 1543                             |
|    | 210° F.....                       | 61.9                               | 63.0                             |
|    | Viscosity Index.....              | 87                                 | 88                               |
|    | Pour Point, °F.....               | -30                                | -5                               |

*Example II*

15 To 138 g. (0.67 mol) of octylphenol is added 57.6 g. (0.67 mol) of vinyl acetate. The mixture is stirred and cooled to 10° C. and concentrated sulfuric acid is added drop-wise to the mixture. 20 A total of 7.3 ml. (0.13 mol) of the acid is employed. The temperature of the reaction mixture rises rapidly to 50° C. where violent boiling occurs. The sulfuric acid is added over a period of approximately 20 minutes and the reaction 25 continued for approximately 3 hours, at which time the product is taken up in 500 ml. of benzene and washed free of acid with water. The water-washed benzene solution is evaporated on a steam bath to remove the benzene and the 30 product dissolved in 823 g. of the mineral lubricating oil described in Example I by heating the mixture with stirring to 140° C. To the heated oil solution is added 100 g. of anhydrous barium hydroxide and 150 ml. of water, the latter being 35 added drop-wise, maintaining a temperature of about 140° C. When the neutralization is complete the product is heated to 175° C. and filtered hot using a filter aid. The product has a sulfate ash of 8.4% and a soap number of 36.7 mg. 40 KOH/g.

A lubricating oil is produced by dissolving a portion of the above product in mineral lubricating oil of the type described in Example I. The resulting oil contains 8.54% by weight of 45 the product and has a sulfate ash of 0.72%. This oil tested in the Lauson engine has a detergency of 80% and bearing weight losses of 2, 12 and 64 mg. at 20, 40 and 60 hours, respectively.

A second lubricating oil is prepared which 50 contains 4.27% by weight of the product of this example and approximately 3.2% of calcium mahogany sulfonate oil concentrate. This oil has a sulfate ash of 0.36% due to the octylphenol vinyl acetate condensation product salt and 55 0.21% due to calcium sulfonate. The oil employed is the same as that used above. Tests on this product in the Lauson engine show the oil to have a detergency of 79% and bearing weight losses of 90, 265 and 408 mg. at 20, 40 and 60 hours, respectively.

A Lauson engine test on the base oil without additives shows a detergency of 58% and bearing weight losses of 175 mg. and 500 mg. at 20 and 40 hours, respectively. Because of severe 65 corrosion, in order to continue the engine operation for the required 60 hours the copper-lead bearings must be removed at 40 hours and replaced with Babbitt bearings.

*Example III*

To 440 g. (2 mols) of nonylphenol dissolved in one liter of naphtha is added 40 ml. (46 g.) of boron trifluoride etherate. The resulting solution is heated to 30° C. and gaseous vinyl chloride is bubbled into the reaction mixture for 75

three hours, at which time approximately 127 g. (2 mols) of vinyl chloride has been used.

The product is cooled, water washed to remove the condensation agent and dissolved in 3000 g. of the mineral lubricating oil described in Example I. The oil solution is heated to evaporate naphtha.

Approximately one-third of the above product is heated to 125° C. and neutralized with calcium hydroxide using 27 g. of calcium hydroxide and approximately 50 ml. of water. The product is heated to 175° C. and filtered. This product is an oil concentrate of the calcium salt of the nonylphenol-vinyl chloride condensation product.

Approximately two-thirds of the condensation product in oil solution is neutralized by treatment with 59 g. of sodium hydroxide and 100 ml. of water. The product is heated to 200° C. and filtered. This product is an oil concentrate of the sodium salt of the nonylphenol-vinyl chloride condensation product.

Approximately one-half of the oil solution of sodium salt as described in the preceding paragraph is diluted with 500 ml. of a light petroleum naphtha and to this solution is added 100 g. of zinc chloride in 250 ml. of isopropanol. The product is heated to evaporate the naphtha and alcohol and then filtered. This product is an oil concentrate of the zinc salt of the nonylphenol-vinyl chloride condensation product.

Lubricating oils are prepared by dissolving 10% by weight of each of the above metal salt concentrates in additional quantities of the mineral lubricating oil described in Example I. Engine tests on these oils show that the condensation product salts impart both detergency and anti-corrosion characteristics to the base oil.

#### Example IV

To 529 g. (3 mols) of o-cyclohexylphenol is added 2 liters of a light petroleum thinner consisting primarily of hexanes and heptanes and 180 g. (2.5 mols) of vinyl ethyl ether. Concentrated sulfuric acid is slowly added to the mixture while maintaining a temperature of about 70° C. A total of 54.4 ml. of the acid is employed. After completing the addition of sulfuric acid the mixture is refluxed for five hours at approximately 72° C. and at this time the product is water washed to remove acid.

The water-washed product is dissolved in 3500 g. of mineral lubricating oil of the type described in Example I and the oil solution heated to evaporate hydrocarbon thinner.

Approximately one-third of the above oil solution of condensation product is treated with 123 g. of lead oxide and 100 ml. of water. The mixture is heated with stirring to 175° C. and then filtered while hot, using a filter aid. The product is an oil concentrate of the lead salt of o-cyclohexylphenol-vinyl ethyl ether condensation product.

Approximately one-third of the oil solution of the condensation product produced as above is neutralized by treatment with freshly precipitated magnesium hydroxide (32 g.) as a slurry in water. The mixture is heated with stirring to 175° C. and filtered to yield an oil concentrate of the magnesium salt of o-cyclohexylphenol-vinyl ethyl ether condensation product.

The remaining one-third portion of the oil solution of the condensation product produced as above is neutralized with lithium hydroxide using approximately 46 g. of the lithium hydroxide

monohydrate in 250 ml. of water. The mixture is heated with stirring to 100° C. and filtered while hot to yield the corresponding lithium salt in oil solution.

Each of the above metal salt concentrates, dissolved in mineral lubricating oil to give products containing approximately 2% by weight of the metal salt, have detergency and anti-corrosion characteristics similar to those of the oil prepared as described in Example I.

#### Example V

A paraffin wax having an average molecular weight of about 350 is treated with gaseous chlorine to obtain a chlorinated paraffin wax containing approximately one atom of chlorine per molecule of the wax. This product is condensed with phenol in the presence of anhydrous aluminum chloride to obtain a wax substituted phenol having a molecular weight of approximately 450.

About 450 g. of the wax substituted phenol prepared as just described is mixed with 86 g. of vinyl acetate and 20 g. of concentrated sulfuric acid is added to the mixture slowly with stirring. The rate of addition is so controlled that the temperature of the reaction mixture is maintained between 70° C. and 80° C. After the addition of sulfuric acid is complete the reaction mixture is maintained at about the same temperature and stirred for an additional two hours. The product is dissolved in one liter of petroleum naphtha and water washed to remove acid. The water-washed product is neutralized with calcium hydroxide in the presence of a small amount of water by refluxing the naphtha solution for three hours. Excess water is removed by continuing the refluxing with a water trap in the reflux line and the dehydrated solution is filtered to remove solids. After evaporation of the naphtha the product consists of the calcium salt of a wax substituted phenol-vinyl acetate condensation product.

A lubricating oil prepared by dissolving 6% by weight of the above product in an SAE 30 mineral lubricating oil having a viscosity index of about 50 has good detergency and exceptional anti-corrosion characteristics as indicated by a bearing weight loss of less than 100 mg. in the Chevrolet engine test.

#### Example VI

To 170 g. of p-phenylphenol in solution in one liter of naphtha is added 34 g. of boron trifluoride etherate. To this mixture is added 86 g. of vinyl isopropyl ether. The ether is added slowly while maintaining a temperature between 20° C. and 30° C. and when the addition is complete the mixture is maintained at room temperature for approximately three hours and then water washed to remove condensation agent.

To the above product is added 1000 g. of mineral lubricating oil and the oil solution is neutralized with 94 g. of anhydrous barium hydroxide using 100 ml. of water. The mixture is heated slowly to 175° C. to remove solvent and water and then filtered. The filtered product consists of an oil concentrate of the barium salt of a phenylphenol-vinyl isopropyl ether condensation product.

A lubricating oil containing approximately 10% by weight of the above oil concentrate operates satisfactorily in heavy duty diesel engine service.

#### Example VII

A 200 g. portion of octylphenol is dissolved in 1000 g. of an SAE 10 solvent refined lubricat-

ing oil having a viscosity index of approximately 85 and to this solution is added 86 g. of vinyl acetate. The mixture is maintained at 75° C. and 10 g. of concentrated sulfuric acid is slowly added. Heating and stirring is continued for approximately 10 hours, at which time the solution is water washed to remove acid.

The product is neutralized by treatment with 174 g. of barium hydroxide octahydrate and gradually heated to 175° C., at which temperature it is filtered. The filtrate is an oil concentrate of the barium salt of an octylphenol-vinyl acetate condensation product. This product, when dissolved in mineral lubricating oil to give an oil containing approximately 3% by weight of the barium salt, imparts detergency and anti-corrosion characteristics to the oil.

*Example VIII*

To 305 g. of m-pentadecylphenol and 57 g. of vinyl acetate in solution in 1500 ml. of a light petroleum naphtha is added 20 g. of concentrated sulfuric acid. The temperature of the reaction mixture rises rapidly to about 80° C. where refluxing occurs. This temperature is maintained for approximately 3 hours and the product then water washed.

The above condensation product is dissolved in 2500 g. of mineral lubricating oil as described in Example I and neutralized with 46 g. of lithium hydroxide monohydrate and 100 ml. of water. The product is heated to 175° C. to remove naphtha and water and filtered while hot. The resulting product is an oil concentrate of the lithium salt of a m-pentadecylphenol-vinyl acetate condensation product. This product, when dissolved in additional quantities of lubricating oil, imparts detergency and anti-corrosion characteristics to the oil.

*Example IX*

Example VIII repeated using carbon tetrachloride in place of light petroleum thinner as the solvent results in a product substantially identical to that obtained with the thinner.

It is to be pointed out that the preceding examples are illustrative of the invention and are not to be considered as limiting because the phenols having one or more of the other hydrocarbon substituents described herein and other vinyl compounds described herein are found to condense under similar conditions to form comparable condensation products. Moreover, the other metals described herein as being useful in preparing the metal salts of the condensation products may be substituted for the metals employed in the examples to give salts which are effective as detergents and anti-corrosion agents when added to mineral lubricating oils. Furthermore, it is to be pointed out that any of the metals described as being useful for the preparation of metal salts of the condensation products are also useful in preparing metal sulfonates and metal sulfonate complexes which cooperate with the additives of this invention to produce non-corrosive lubricating oils of exceptionally high detergency. Such metal sulfonates or metal sulfonate complexes, when used in conjunction with the additives of this invention, are used in amounts between about 0.5% and about 10% based on the finished oil.

I claim:

1. A mineral lubricating oil containing between about 0.05 and about 20% by weight of an oil-soluble metal salt of the acidic condensation prod-

uct of a hydrocarbon substituted phenol, in which the hydrocarbon substituent contains between about 4 and about 30 carbon atoms, and a vinyl compound selected from the class consisting of divinyl ether, vinyl ethyl ether, vinyl propyl ether, vinyl esters of hydrohalogen acids and vinyl esters of fatty acids containing between 1 and 6 carbon atoms in the fatty acid radical, said condensation product being obtained by condensing said phenol with said vinyl compound in the molar ratio of between 0.5 and 3 to 1 at temperatures between about -20° C. and about 150° C.

2. A mineral lubricating oil containing between about 0.05 and about 20% by weight of an oil-soluble alkaline earth metal salt of the acidic condensation product of a hydrocarbon substituted phenol, in which the hydrocarbon substituent contains between about 4 and about 30 carbon atoms, and a vinyl compound selected from the class consisting of divinyl ether, vinyl ethyl ether, vinyl propyl ether, vinyl esters of hydrohalogen acids and vinyl esters of fatty acids containing between 1 and 6 carbon atoms in the fatty acid radical, said condensation product being obtained by condensing said phenol with said vinyl compound in the molar ratio of between 0.5 and 3 to 1 at temperatures between about 0° C. and about 100° C.

3. A mineral lubricating oil containing between about 0.05 and about 20% by weight of an oil-soluble alkali metal salt of the acidic condensation product of a hydrocarbon substituted phenol in which the hydrocarbon substituent contains between about 4 and about 30 carbon atoms and a vinyl compound selected from the class consisting of divinyl ether, vinyl ethyl ether, vinyl propyl ether, vinyl esters of hydrohalogen acids and vinyl esters of fatty acids containing between 1 and 6 carbon atoms in the fatty acid radical, said condensation product being obtained by condensing said phenol with said vinyl compound in the molar ratio of between 0.5 and 3 to 1 at temperatures between about -20° C. and about 150° C.

4. A mineral lubricating oil according to claim 1 in which the molar ratio of phenol to vinyl compound is between 0.8 and 2 to 1.

5. A mineral lubricating oil according to claim 2 in which said alkaline earth metal salt is a barium salt.

6. A mineral lubricating oil according to claim 2 in which said alkaline earth metal salt is a calcium salt.

7. A lubricating oil according to claim 3 in which said alkali metal salt is a lithium salt.

8. A lubricating oil according to claim 3 in which said alkali metal salt is a sodium salt.

9. A mineral lubricating oil containing between about 0.05% and about 20% by weight of an oil-soluble metal salt of the acidic reaction product obtained by condensing at a temperature between 0° C. and 100° C. a hydrocarbon substituted phenol in which the hydrocarbon substituent contains between about 4 and about 30 carbon atoms with vinyl acetate using a molar ratio of phenol to vinyl acetate of between 0.8 and 2 to 1.

10. A mineral lubricating oil containing between about 0.05% and about 20% by weight of an oil-soluble metal salt of the acidic reaction product obtained by condensing cyclohexyl phenol with vinyl ethyl ether using a molar ratio of phenol to vinyl ethyl ether of between 0.8 and 2 to 1, the condensation being effected at temperatures between 0° C. and 100° C.

11. A mineral lubricating oil containing be-

13

tween about 0.05% and about 20% by weight of an oil-soluble metal salt of the acidic reaction product obtained by condensing a hydrocarbon substituted phenol in which the hydrocarbon substituent contains between about 4 and about 30 carbon atoms with vinyl chloride, at a temperature between about 0° C. and about 100° C., using a molar ratio of phenol to vinyl chloride between 0.8 and 2 to 1.

12. A mineral lubricating oil containing between about 0.5% and about 10% by weight of the barium salt of the acidic condensation product obtained by condensing, at temperatures between about 0° C. and about 100° C., approximately equal molar proportions of an alkyl substituted phenol and vinyl acetate, the alkyl substituent of said phenol containing between about 4 and about 30 carbon atoms.

13. A mineral lubricating oil containing between about 0.5% and about 10% by weight of the barium salt of the acidic condensation product obtained by condensing approximately equal molar proportions of octylphenol and vinyl ace-

14

tate at temperatures between about 0° C. and about 100° C.

14. A mineral lubricating oil according to claim 1 containing also between about 0.5% and about 10% by weight of an oil-soluble metal sulfonate.

15. A mineral lubricating oil according to claim 1 containing also between 0.5% and 10% of a modified sulfonate prepared by heating an oil-soluble metal sulfonate with an inorganic base selected from the class consisting of metal oxides, hydroxides, carbonates and bicarbonates to solubilize said base, said modified sulfonate having a ratio of equivalents of metal to equivalents of sulfonic acids between 1.1 and 3 to 1.

LOREN L. NEFF.

## References Cited in the file of this patent

## UNITED STATES PATENTS

| 20 | Number    | Name           | Date          |
|----|-----------|----------------|---------------|
|    | 2,307,885 | Gleason        | Jan. 12, 1943 |
|    | 2,375,222 | Griffin et al. | May 8, 1945   |
|    | 2,422,276 | Mikeska        | June 17, 1947 |